# EUROPEAN PATENT SPECIFICATION

(11) **EP 3 394 342 B1**
(45) Date of publication and mention of the grant of the patent: **14.02.2024**
(21) Application number: 16825737.6
(22) Date of filing: 21.12.2016
(51) Int. Cl.: D21H 25/00, D21H 27/10, D21H 27/30, D21H 19/82, D21H 19/84, D21H 17/17, D21H 17/35, D21H 17/67

(54) **RAINPROOF PAPER SACK**
REGENDICHTER PAPIERSACK
SAC EN PAPIER IMPERMÉABLE

(30) Priority: 21.12.2015 EP 15201668
(43) Date of publication of application: 31.10.2018
(73) Proprietor: Billerud Aktiebolag (publ), 169 27 Solna (SE)
(72) Inventor: LINDSTRÖM, Ove, SE-952 91 Kalix (SE)
(74) Representative: Kransell & Wennborg KB
(86) International application number: PCT/EP2016/082115
(87) International publication number: WO 2017/108910

(56) References cited:
- EP-A1- 0 718 437
- WO-A1-98/57861
- WO-A1-99/02772
- WO-A1-03/010055
- WO-A1-2011/000942
- WO-A1-2013/069788
- WO-A1-2013/164646
- DE-T2-602005 003 089
- US-A1- 2003 226 648

## Description

### TECHNICAL FIELD

The present disclosure relates to a rainproof paper sack suitable for a hydraulic binder, such as cement, as well as a sack paper for use as the outer ply of such a rainproof sack.

### BACKGROUND

During filling and storage of powdery material, such as cement, paper sacks are required to meet high standards.

Firstly, the paper sacks need to hold a considerable material weight, i.e. have high tensile strength. For this purpose, Kraft paper is a suitable sack wall material. The sacks typically have two or more walls, i.e. layers of paper material, to further strengthen the sack construction. A wall layer of a sack is often referred to as a ply. Production of ply material (i.e. sack paper) is for example disclosed in WO 99/02772.

Secondly, a material such as cement is sensitive to moisture contamination during storage. Hence, cement sacks often require a protection against atmospheric water vapor penetration through the sack plies. Such protection is often achieved by a moisture barrier incorporated as an intermediate layer in the sack, i.e. between two plies of the paper material. The moisture barrier is typically a plastic film ("free film"), e.g. of polyethylene (PE), that is impermeable to water. The free film may also improve resistance to grease and prevent contamination by microorganisms.

Thirdly, the paper sack should vent air during filling. In detail, the air that accompanies the powdered material shall efficiently vent from the sack as the filling machines that delivers the material run at high throughput rates. Often, the venting capability of the sack is the actual limiting factor for the filling rate. Efficient venting also prevents air from being trapped in the sack. Such trapped air may otherwise cause under-weight packs, sack rupture and problems when sacks are stacked for transportation. The "venting" is also referred to as "deaeration".

During the filling process, the only way for air to escape from the interior of the sack has, in many sack constructions, been through the walls of the sack. Kraft paper of high porosity is often used in the walls to achieve air permeability. However, an increased porosity of the paper normally results in a decrease in the overall strength. In particular, the strength may be significantly reduced if holes must be made in the paper material to achieve sufficient air permeability. Furthermore, the use of a free film may reduce deaeration during filling, since most such films are impermeable to air. Therefore, the free film layer has been provided with slits or perforations to facilitate deaeration.

WO 2013/164646 discloses a coated fibre-based material comprising a fibre-based substrate comprising microfibrillated cellulose and having at least first and second barrier coatings formed thereon. It further discloses articles such as paper products, particularly food grade packaging, formed from said coated material, and to methods of preparing said coated material and paper products.

WO2011/000942 discloses a material suitable for a ply of a sack, comprising a porous sheet provided with a coating on at least one of its surfaces, wherein said coating comprises at least one polyolefin. It further discloses a sack comprising a ply, which comprises such a material.

DE602005003089 T2 discloses a bag that has a polyethylene film that is impermeable to air and interposed between two paper folds. The film is folded to form a sleeve with two contactless edges spaced by an interval for permitting free passage of the air for deaeration, during filling of the bag. The fold has a band impermeable to air to impose a path to the air such that air penetrates between the fold and the film, and evacuates towards outside.

### SUMMARY

An object of the present disclosure is to provide a sack that is rainproof and still meet other requirements of the sack industry. Examples of such other requirements are strength (to prevent rupture during handling), deaeration during filling (to allow high filling rates) and cost efficiency.

Another object of the present disclosure is to provide a sack paper for use as the outermost ply of the rainproof sack.

The present disclosure presents a coated paper for use in a sack, wherein: the coated paper comprises a paper layer that is internal-sized with at least one hydrophobic size;
the sized paper layer is creped;
the sized paper layer is provided on a first side with a pre-coating layer and a barrier coating layer;
the pre-coating layer comprises binder and inorganic filler in a dry weight ratio of between 10:100 and 50:100;
the barrier coating layer comprises clay and synthetic rubber in a dry weight ratio between 1:1 and 2.4:1;
the sized paper is provided on a second side with a backside coating layer, which backside coating may have a coat weight of 1-5 g/m², such as 2-4 g/m²; and
the grammage according to ISO 536 of said coated paper is 75-140 g/m², such as 80-115 g/m²,
wherein the particle size (% < 2 µm) of the inorganic filler is 80 or less.

In an embodiment the backside coating comprises starch and/or rubber. The rubber may be synthetic rubber, such as styrene-butadiene rubber.

In an embodiment the inorganic filler of the pre-coating layer comprises or consist of CaCO₃ pigment.

In an embodiment the binder of the pre-coating is selected from a starch and a rubber, such as a synthetic rubber.

In an embodiment the pre-coating layer comprises binder and inorganic filler in a dry weight ratio of between 15:100 and 40:100, such as between 20:100 and 35:100.

In an embodiment the inorganic filler accounts for at least 70 % of the dry weight of the pre-coating layer.

In an embodiment the particle size (% < 2 µm) of the inorganic filler is between 50 and 80, such as between 50 and 75, such as between 55 and 75.

In an embodiment the pre-coating layer comprises a thickening agent, such as CMC.

In an embodiment the coat weight of the pre-coating layer is 5-12 g/ m², such as 6-10 g/m².

In an embodiment the coat weight of the barrier coating layer is 5-15 g/m², such as 6-12 g/m², such as 7-10 g/m².

In an embodiment the barrier coating layer comprises styrene-butadiene rubber.

In an embodiment the synthetic rubber of the barrier coating layer is provided in the form of latex.

In an embodiment the barrier coating layer comprises a platy clay, such as platy kaolin.

In an embodiment the at least one hydrophobic size comprises rosin size.

In an embodiment the at least one hydrophobic size comprises AKD or ASA.

In an embodiment the at least one hydrophobic size comprises AKD and rosin size.

In an embodiment the sized paper layer has been sized with AKD and rosin size in a weight ratio between 1:6 and 1:1.5, such as between 1:5 and 1:2.

In an embodiment the Cobb 1800 s value measured according to ISO 535 of the sized paper layer is less than 60 g/m², such as less than 50 g/m², such as less than 45 g/m², such as less than 40 g/m².

In an embodiment the Cobb 60 s value measured according to ISO 535 of the sized paper layer is less than 30 g/m², such as less than 25 g/m².

In an embodiment the sized paper layer is a bleached paper layer.

In an embodiment brightness of the sized paper layer is at least 78 %, such as at least 83 %, according to ISO 2470-1.

In an embodiment the sized paper layer is a Kraft paper ply.

In an embodiment the sized paper layer is formed from a paper pulp comprising at least 50 dry weight % softwood pulp, such as at least 75 dry weight % softwood pulp, such as at least 90 dry weight % softwood pulp.

In an embodiment the grammage according to ISO 536 of the sized paper layer is 60-90 g/m².

The present disclosure also presents a sack for a hydraulic binder comprising an outer ply composed of the coated sack paper.

### BRIEF DESCRIPTION OF THE DRAWINGS

Fig 1 shows a sack according to the present disclosure configured to allow "top deaeration".
Fig 2 shows the sack of Fig 1 provided with a top patch for reinforcement.

### DETAILED DESCRIPTION

As a first, non-claimed, aspect there is provided a multi-ply sack comprising an inner paper ply and an outer paper ply, wherein the outer paper ply comprises a paper layer that is sized with at least one hydrophobic size. Further and the outside of the sized paper layer is provided with a pre-coating layer and a barrier coating layer.

The outside of the outer paper ply is exposed to the surroundings, which means that the outside of the outer paper ply can be exposed to rain.

Bleached paper is generally significantly less hydrophobic than unbleached paper. Accordingly, bleached/white sack paper has higher water absorptiveness and is more sensitive to rain. Therefore, it is more challenging to develop a rainproof sack having a bleached outer paper ply than a rainproof sack having an unbleached outer paper ply. Still, sacks having white outer plies are demanded on the marked, also for sacks that may be exposed to rain. The concept of the present disclosure is thus particularly beneficial when the sized paper layer of the outer paper ply is bleached. The brightness of the sized paper layer may for example be at least 78 % or at least 80 % according to ISO 2470-1. Preferably, it is at least 83 %.

The total amount of hydrophobic size used for sizing the sized paper layer may for example be 1.5-4.0 kg/ton paper, such as 2.0-3.5 kg/ton paper. The sizing technique may be internal sizing, which means that the size is added in the wet end of the paper machine, or surface sizing, which means that the size is applied to the paper surface after initial drying. Examples of hydrophobic sizes are alkylketene dimer (AKD), alkenylsuccinic anhydride (ASA) and rosin size, which are all commercially available papermaking chemicals. The inventor has found that AKD and ASA reduce the water absorptiveness more efficiently than rosin size. However, the inventor has also noted that the hydrophobicity of a paper sized with ASA may deteriorate after longer storage times due to sensitivity to oxygen and sunlight. The inventor concludes that sizing with a combination of AKD and rosin size may be preferred. The added amount of AKD may be 0.4-1.4 kg/ton paper and preferably 0.5-1 kg/ton paper. The added amount of rosin size may be 1.2-4.2 kg/ton paper and preferably 1.5-3 kg/ton paper. The weight ratio of AKD to rosin size may be between 1:6 and 1:1.5. Preferably, the weight ratio is between 1:5 and 1:2 and more preferably between 1:4 and 1:2.5.

In the context of the present disclosure, "kg/ton paper" refers to kg per ton of dried paper from the paper making process. Such dried paper normally has a dry matter content (w/w) of 90-95 %.

Alum may also be added to the pulp, e.g. in an amount of 0.5-5 kg/ton paper. The addition of alum is particularly beneficial when the hydrophobic size comprises rosin size. Alum refers to hydrated potassium aluminium sulphate (potassium alum).

The Cobb value represents the amount of water absorbed by a paper surface in a given time. Consequently, the hydrophobic sizing reduces the Cobb value of the sized paper layer. Two examples of Cobb values are Cobb 60 s and Cobb 1800 s, wherein the absorption of water is measured after 60 seconds and 1800 seconds (30 minutes), respectively.

Rain typically means long-term exposure to rain and therefore, the Cobb 1800 s for the outside of the sized paper layer is considered to be particularly relevant.

The Cobb 1800 s value measured according to ISO 535 of the outside of the sized paper layer may for example be less than 60 g/m². Preferably it is less than 50 g/m² and more preferably less than 45 g/m² or less than 40 g/m². A typical lower limit for the Cobb 60 s value may be 25 or 30 g/m². A preferred range for the Cobb 1800 s value is thus 25-50 g/m².

The Cobb 60 s value measured according to ISO 535 of the outside of the sized paper layer may for example be less than 30 g/m². Preferably it is less than 25 g/m². A typical lower limit for the Cobb 60 s value may be 10 or 15 g/m². A preferred range for the Cobb 60 s value is thus 15-25 g/m².

It is to be understood that the Cobb values are measured on the surface of sized paper layer before it is coated.

The sizing merely reduces water absorption. It does not completely prevent it. Therefore, the sized paper layer is provided the barrier coating layer (further discussed below).

As the outer paper ply is coated with a barrier coating layer, the sack of the first aspect may lack a plastic film arranged between the outer paper ply and the inner paper ply. Such a plastic film, which is also referred to as a "free film", is often used in prior art sacks to provide a barrier for moisture and liquid water.

Between the sized paper layer and the barrier coating layer, the pre-coating layer is provided. A purpose of the pre-coating layer is to even the surface of the sized paper layer and thus reduce the amount of barrier material needed to form an efficient barrier coating layer. This is particularly beneficial when the sized paper layer is creped.

However, the reduction in the amount of barrier material is only a cost reduction if the pre-coating material is cheaper than a typical barrier material. Therefore, the pre-coating layer comprises a high amount of (relatively cheap) inorganic filler. In addition, the pre-coating layer comprises a binder to hold the pre-coating layer together and bind it to the sized paper layer.

The binder and the inorganic filler are provided in a dry weight ratio of between 10:100 and 50:100 (sometimes referred to as between 10 and 50 parts). Preferably, the pre-coating layer comprises binder and inorganic filler in a dry weight ratio of between 15:100 and 40:100. The most preferred dry weight ratio is between 20:100 and 35:100. A benefit of a relatively high proportion of binder (i.e. ≥ 20 parts) is that the pre-coating better contributes to the overall barrier properties of the outer paper ply.

The filler and the binder are preferably the main components of the pre-coating layer. The inorganic filler normally accounts for at least 70 % of the dry weight of the pre-coating layer.

Preferably, the particles of the inorganic filler are relatively large. Coarser particles means lower specific surface area, which in turn means that the binder in the pre-coating can form a more robust film. At the same time, the coarser particles do not negatively affect the printing properties as a barrier coating covers the pre-coating. Further, filler products with coarser particles are generally cheaper. Yet other benefits of coarser particles is that they result in a pre-coating layer that better cover the surface and better prevents formation of blade scratches during blade coating of a barrier layer comprising platy clay than a pre-coating layer with finer particles.

The particle size of filler and pigment is often expressed as the weight proportion of particles having a particle size below 2 µm. The value (% < 2 µm) is often measured using the particle size analyzer SediGraph 5100 (micromeritics^{®}).

When filler/pigment is used in coatings to improve printing properties, the particle size value (% < 2 µm) is generally above 80. In contrast, the particle size value (% < 2 µm) of the inorganic filler of the present disclosure is preferably 80 or lower, such as between 50 and 80. In some embodiments, the particle size value (% < 2 µm) is between 50 and 75, such as between 55 and 75.

The inorganic filler may for example comprise or consist of CaCO₃ pigment. Other types of filler are generally more expensive.

The binder of the pre-coating can for example be starch or rubber, such as a synthetic rubber. Rubber is preferred as it makes a contribution to the water barrier properties of the outer paper ply. The rubber may for example be a synthetic rubber, preferably styrene-butadiene rubber.

When preparing a composition form forming the pre-coating layer, the synthetic rubber is normally provided in the form of a water dispersion, normally referred to as latex.

Examples of other (optional) components of the pre-coating layer are thickening agents, coloring agents, optical brightening agents and antifoaming agents. One embodiment of the pre-coating layer comprises carboxymethyl cellulose (CMC), which is a thickening agent. A synthetic thickener, such as an acrylic copolymer, can also be used. An example of synthetic thickener is Rheocoat 35 from Coatex.

The coat weight of the pre-coating layer may for example be 5-12 g/m², such as 6-10 g/m². If the coat weight of the pre-coating is too low, higher amounts of barrier material, which is expensive, are needed in the next coating layer to obtain an effective barrier layer. If the coat weight of the pre-coating is too high, the cost of the product will be unnecessarily high.

In embodiments of the present disclosure, the barrier coating layer comprises a synthetic rubber, such as styrene-butadiene rubber. When preparing the barrier coating composition, the synthetic rubber is normally provided in the form of latex.

In alternative or complementary embodiments of the present disclosure, the barrier coating layer comprises a clay, preferably a platy clay, such as platy kaolin. The most preferred type of clay is hyper-platy kaolin.

Clay (and in particular hyper-platy clay) creates a tortous path for moisture transmission and therefore suitable for creating barrier functions.

A specific example of hyper-platy kaolin is the product Barrisurf^{™} (Imerys).

A barrier coating layer consisting of synthetic rubber is sometimes difficult to print. In a preferred embodiment, the barrier coating layer thus comprises both the synthetic rubber and the clay. For example, the synthetic rubber and the platy clay may account for at least 50 %, such as at least 75 or 85 %, of the dry weight of the barrier coating layer. The dry weight ratio of clay to synthetic rubber may for example be between 1:1 and 2.4:1, such as between 1.3:1 and 2.1:1.

The barrier coating layer may comprise a thickening agent, such as CMC or a synthetic thickener, such as an acrylic copolymer. As mentioned above, an example of a synthetic thickener is Rheocoat 35 from Coatex.

The coat weight of the barrier coating layer may for example be 5-15 g/m², such as 6-12 g/m², such as 7-10 g/m². If the coat weight is too low, the barrier coating layer may fail to provide an efficient barrier. If the coat weight is too high, the cost of the product will be unnecessarily high. It is notable that the barrier chemicals are generally relatively expensive.

In embodiments of the first aspect, the inside of the sized paper layer is provided with a backside coating. A purpose of such a backside coating is to prevent curling that can otherwise occur when paper coated on one side only is dried. To contribute to the overall water resistance of the outer paper ply, the backside coating may comprise a barrier chemical, such as rubber. Again, synthetic rubber, such as styrene-butadiene rubber, is preferred. As a complement or an alternative to the barrier chemical, the backside coating may comprise starch.

The coat weight of the backside coating is preferably 1-5 g/m², such as 2-4 g/m².

To provide strength, the sized paper layer of the outer paper ply is preferably a Kraft paper, which means that is formed from a pulp prepared according to the Kraft process. For the same reason, the starting material used for preparing the pulp that is used for forming the sized paper layer of the outer paper ply can comprise softwood (which has long fibers and thus forms a strong paper). Accordingly, the sized paper layer is preferably formed from a paper pulp comprising at least 50 % softwood pulp, preferably at least 75 % softwood pulp and more preferably at least 90 % softwood pulp. The percentages are based of the dry weight of the pulp.

A sack paper normally has a grammage according to ISO 536 of 50-140 g/m². A sack paper of a higher grammage is stronger, but also more expensive. For the sized paper layer of the outer paper ply of the present disclosure, the grammage is preferably 60-125 g/m² and more preferably 65-100 g/m². For the outer paper ply (including the coating layers), the grammage according to ISO 536 is preferably 65-150 g/m², such as 75-140 g/m², such as 80-115 g/m².

The tensile strength is the maximum force that a paper will withstand before breaking. In the standard test ISO 1924-3, a stripe having a width of 15 mm and a length of 100 mm is used with a constant rate of elongation. The tensile strength is one parameter in the measurement of the tensile energy absorption (TEA). In the same test, the tensile strength, the stretchability and the TEA value are obtained.

TEA is sometimes considered to be the paper property that best represents the relevant strength of the paper sack wall. This is supported by the correlation between TEA and drop tests. When a sack is dropped, the filling goods move inside the sack when it hits the floor. This movement means a strain on the sack wall. To withstand the strain, the TEA should be high, which means that a combination of high tensile strength and good stretch in the paper will then absorb the energy.

The stretchability according to ISO 1924-3 of the sized paper layer or the outer paper ply may for example be at least 4.5 % in the machine direction (MD) and at least 5.5 % in the cross direction. To obtain high stretchability in the MD, the sized paper layer may be creped.

For example, the sized paper layer may be creped by a Clupak or Expanda unit. The skilled person knows how to adjust such a unit to obtain a desired stretchability in the MD.

The TEA index is the TEA value divided by the grammage. The TEA according to ISO 1924-3 of the outer paper ply may for example be 150-300 J/m² in both MD and CD. The TEA index according to ISO 1924-3 of the outer paper ply may for example be 2.2-3.5 J/g in the MD and 2.8-4.2 J/g in the CD.

The tear strength according to ISO 1974 of the sized paper layer or the outer paper ply may for example be at least 840 mN, such as at least 950 mN in both the machine direction (MD) and in the cross direction (CD). In one embodiment, the tear strength is at least 860 mN in MD and at least 1000 mN in CD.

To obtain satisfactory strength, the sized paper layer may comprise starch. For example, the added amount of starch may be 1-15 kg/ton paper, such as 2-12 kg/ton paper, such as 4-11 kg/ton paper. The starch may for example be a cationic starch or a mixture of cationic and anionic starch.

To allow for sufficient deaeration, the Gurley porosity according to ISO 5636-5 of the inner paper ply is less than 10 s. Preferably, it is less than 8 s and more preferably less than 6 s. Brown QuickFill Plus and Brown QuickFill SE, which are marketed by BillerudKorsnäs and have Gurley porosities of 3 s and 5 s, respectively, are examples of sack papers that can be used for the inner paper ply. Normally, it is pointless to reduce the Gurley value below 2.5 s. Further, it is generally difficult to produce a sack paper of such a low Gurley value and sufficient strength. Ranges for the Gurley porosity of the inner paper ply are thus 2.5-10 s, 2.5-8 s and 2.5-6 s.

To provide strength, the inner paper ply is preferably a Kraft paper ply. For the same reason, the starting material used for preparing the pulp that is used for forming the paper of the inner paper ply can comprise softwood. Accordingly, the inner paper ply is preferably formed from a paper pulp comprising at least 50 % softwood pulp, preferably at least 75 % softwood pulp and more preferably at least 90 % softwood pulp. The percentages are based of the dry weight of the pulp.

As explained above, sack paper normally has a grammage according to ISO 536 of 50-140 g/m² and a sack paper of a higher grammage is stronger, but also more expensive. For the inner paper ply of the present disclosure, the grammage is preferably 55-100 g/m² and more preferably 60-90 g/m².

The inner paper ply preferably provides substantial dry strength to the sack. Accordingly, the tensile energy absorption (TEA) according to ISO 1924-3 of the inner paper ply is preferably at least 175 J/m² in the machine direction (MD). In the cross direction (CD), the TEA according to ISO 1924-3 is preferably at least 182 J/m².

More preferably, the TEA according to ISO 1924-3 is at least 196 J/m² in the MD and/or at least 203 J/m² in the CD.

A typical upper limit for the TEA may be 260 J/m² in MD and 270 J/m² in CD.

To take the TEA in both MD and CD into account, a geometric TEA may be calculated as the square root of the product of TEA in MD and TEA in CD (TEA (geometric) = V(TEA (MD) * TEA (CD))).

Accordingly, the geometric TEA according to ISO 1924-3 of the inner paper ply is preferably at least 178 J/m², such as 178-265 J/m², and more preferably 199-265 J/m².

To reduce the fibre consumption, the inner paper ply is advantageously strong already at a relatively low grammage. Therefore, the TEA index according to ISO 1924-3 of the inner paper ply may be at least 2.5 J/g in the MD and at least 2.6 J/g in the CD. Preferably, the TEA index according to ISO 1924-3 of the inner paper ply is at least 2.8 J/g, such as 2.8-3.5 J/g in the MD and at least 2.9 J/g, such as 2.9-3.9 J/g in the CD.

The porosity of the inner paper ply of the sack of the present disclosure allows air to pass from the inside of the sack to an interspace between the inner paper ply and the outer paper ply. Further, the sack of the present disclosure is configured to allow air to escape from the interspace between the inner paper ply and the outer paper ply (to the ambient air) during filling of the sack.

Preferably, the sack design is such that air can escape from the interspace between the inner paper ply and the outer paper ply through a top end of the sack during filling of the sack.

For example, a top end of the sack may be formed by folding and gluing the plies such that a portion of the top end is not sealed and air can escape from the interspace through the non-sealed portion during filling of the sack. Such an embodiment is further discussed below with reference to figures 1 and 2.

The sack of the present disclosure is preferably a valve sack. Valve sacks are well known to the skilled person. A valve sack is provided with a valve through which it may be filled. Such a valve is normally provided at a folded top end of the sack. A typical valve is further discussed below with reference to figures 1 and 2.

Figure 1 illustrates a multi-ply sack 100 according to an embodiment of the present disclosure having a top end 111 and a bottom end 112. The sack comprises an inner paper ply 101 and an outer paper ply 102. To improve rain resistance, the paper layer of the outer paper ply 102 is sized with at least one hydrophobic size. Further, the paper layer is coated with a pre-coating and a barrier coating. To facilitate deaeration, the Gurley porosity according to ISO 5636-5 of the inner paper ply 101 is less than 10 s.

The sack 100 is configured to allow air to escape (the air escape is illustrated by the arrow 103) from an interspace between the inner paper ply 101 and the outer paper ply 102 through the top end 111 of the sack 100 during filling of the sack 100. Such a deaeration is achieved by a non-sealed portion 104 forming an opening between the inner paper ply 101 and the outer paper ply 102 at the top end 111. The non-sealed portion 104 may be flanked by sealed portions 105, i.e. portions in which the outer paper ply 102 is sealed (preferably glued) to the inner paper ply 101. For a 25 kg sack 100 having a width of 400-420 mm, the width of the non-sealed portion may for example be 150-160 mm and for a 35 kg having a width of 440-460 mm, the width of the non-sealed portion maybe 190-200 mm.

The top end 111 of the sack 100 of figure 1 further has a filling valve 106 into which a filling spout may be inserted. The arrow 107 illustrates how the filling spout is inserted into the valve 106. A ceiling of the valve 106 is reinforced by a valve reinforcement 108, which preferably is composed of paper. Because of the reinforcement provided by the valve reinforcement 108, the sack 100 can hang on the filling spout during filling without breaking. When fully opened, the opening of the valve 106 may be approximatively diamond-shaped.

Figure 2 illustrates the sack 100 of figure 1 onto which a top patch 201 has been applied. The top patch reinforces top end 111 of the sack 100. A slit 202 in the top patch 201 ensures that the air still can escape through the non-sealed portion 104 during filling. The slit 202 is thus substantially aligned with the non-sealed portion 104. Further, the width of the slit 202 is preferably approximately the same as the width of the non-sealed portion 104. Again, the escape of air from the interspace between the inner paper ply 101 and the outer paper ply 102 through the top end 111 of the sack 100 is illustrated by the arrow 103.

To best protect the contents against rain, the sack 100 is oriented such that the opening formed by the non-sealed portion 104 is facing down.

The dimensions of the sack of the present disclosure may for example be such that it has a volume of 8-45 liters, preferably 12-45 liters in a filled configuration.

The sack of the present disclosure may for example contain a hydraulic binder, such as cement. The amount of the hydraulic binder may for example be 17-60 kg. 25 kg sacks, 35 kg sacks and 50 kg sacks are demanded on the market and may thus be prepared according to the present disclosure. The dimensions of a filled 25 kg sack may for example be 400×450×110 mm. A "25 kg sack" typically can be filled with about 17.4 liters of material, while a "50 kg sack" is typically can be filled with about 35 liters of material.

As a second aspect of the present disclosure, there is provided a coated paper for use in a sack, wherein
the coated paper comprises a paper layer that is internal-sized with at least one hydrophobic size;
the sized paper layer is creped;
the sized paper layer is provided on a first side with a pre-coating layer and a barrier coating layer;
the pre-coating layer comprises binder and inorganic filler in a dry weight ratio of between 10:100 and 50:100;
the barrier coating layer comprises clay and synthetic rubber in a dry weight ratio between 1:1 and 2.4:1;
the sized paper is provided on a second side with a backside coating layer; and
the grammage according to ISO 536 of said coated paper is 75-140 g/m², such as 80-115 g/m²,
wherein the particle size (% < 2 µm) of the inorganic filler is 80 or less.

The second aspect is a preferred embodiment of the outer paper ply of the first, non-claimed, aspect. The embodiments of the outer paper ply of the first, non-claimed, aspect discussed above apply *mutatis mutandis* to the coated paper of the second aspect.

### EXAMPLES

### Preparation of a sized paper layer, trial 1

Bleached kraft papers having a grammage of 70 or 80 g/m² for use as a sized paper layer according to the present disclosure were prepared as follows.
Type of pulp: Bleached sulphate pulp from softwood
HC refining: 180 kWh/ton paper
LC refining: 100 kWh/ton paper
Pulp additive: 2.5 kg/ton paper of Fennosize G516/9M (a mixture of AKD and rosin size in a weight ratio of 1:3)
Pulp additive: 1.0 kg/ton paper of Raisamyl 50021, 1.0 kg/t (cationic starch)
Pulp additive: 15.0 kg/ton paper of Fennostrength UF 3467 (urea-
formaldehyde wet strength agent)
Pulp additive: 0.42 kg/ton paper of Eka NP 247 (retention nano particle)
Pulp additive: 0.07 kg/ton paper of Eka PL 1510U (retention polymer)
Pulp additive: 0.5-2.5 kg/ton paper of Kemira ALG (alum) to obtain a headbox pH of 4.8-4.9

As specified above, a wet strength agent was added. This is however not necessary when preparing a sized paper layer according to the present disclosure because the sized paper layer is coated to prevent soaking.

Wet creping was carried out to increase the stretchability in the MD.

The properties of the prepared bleached kraft papers (BKP70 and BKP80) and a reference paper are presented in table 1 below.

**Table 1.**

| | BKP80 Bleached | BKP70 Bleached | SplashBag* Unbleached (as tested) | SplashBag* Unbleached (as specified) |
|---|---|---|---|---|
| Grammage (g/m²) | 80 | 70 | 70 | 70 |
| TEA index MD/CD (J/g) | 2.8/3.6 | 2.7/3.2 | 3.1/3.7 | 3.1/3.4 |
| Stretchability MD/CD (%) | 6.0/9.2 | 7/8.7 | 6.1/8.4 | 5.8/8.0 |
| Tear strength MD/CD (mN) | 1200/ 1120 | 1050/ 1092 | 700/700 | 749/798 |
| Wet tensile strength MD (kN/m) | 1.74 | 1.24 | 1.97 | 1.8 |
| Cobb 60 s (g/m²) | 21 | 20 | N/A | 21 |
| Cobb 1800 s (g/m²) | 39 | 38 | 40 | N/A |
| Gurley (s) | 22 | 22 | N/A | N/A |

| | | | | |
|---|---|---|---|---|
| *"SplashBag" refers to the outer ply of a SplashBag marketed by Mondi. | | | | |

In table 1, it is seen that the Cobb 1800 s values of BKP70 and BKP80 are lower than the Cobb 1800 s value of the outer layer of the Mondi SplashBag even though BKP70 and BKP80 are bleached and the outer layer of Mondi SplashBag is unbleached. This is of significance as the Cobb 1800 s value reflects the rain resistance of the paper.

### Preparation of a sized paper layer, (prophetic) trial 2

Bleached kraft paper having a grammage of 80 g/m² for use as a sized paper layer according to the present disclosure is prepared as follows.
Type of pulp: Bleached sulphate pulp from softwood
HC refining: 180 Wh/ton paper
LC refining: 80 kWh/ton paper
Pulp additive: 2.5 kg/ton paper of Fennosize G517/9M (a mixture of AKD and rosin size in a weight ratio of 1:3)
Pulp additive: 7.0 kg/ton paper of Roquette Hi-Cat 5216 A (cationic starch)
Pulp additive: 3.0 kg/ton paper of Roquette Vector AS 104 (anionic starch)
Pulp additive: 0.5-2.5 kg/ton paper of Kemira ALG (alum) to obtain a headbox pH of 5.6-5.9

Wet creping was carried out to increase the stretchability in the MD.

### Preparation of a coated sack paper for an outer paper ply

To prepare a coated sack paper for an outer paper ply according to the present disclosure, an aqueous pre-coating composition comprising styrene-butadiene latex and CaCO₃ pigment in a dry weight ratio of 30:100 is prepared. CMC (thickening agent) is added to the pre-coating composition such that a viscosity of about 700 cP (measured according to Scan-P 50:84, but with a sample temperature of 34-40 °C) is obtained. Further, the pH of the pre-coating composition is adjusted to 8.3 using NaOH.

The pre-coating composition is then applied to sized paper prepared according to trial 2 above using a blade coater. The pressure and angle of the coating blade is adjusted such that the coat weight of the pre-coating is 8 g/m².

Further, an aqueous backside coating composition comprising starch (4-6 %) and styrene-butadiene latex (2-5 %) is prepared. The backside coating composition is applied to the backside of the paper via a roll distributing system at the same position as the coater or the pre-coating, i.e. opposite of the blade, to obtain a backside coat weight of 2-4 g/m².

The pre-coating is dried with IR-heaters and drying cylinders to such an extent that the barrier coating composition (described below) can be applied without problems like scuffing of the pre-coating.

An aqueous barrier coating composition comprising styrene-butadiene latex and hyper-platy kaolin pigment (Barrisurf^{™} (Imerys)) in a dry weight ratio of 50:100 is prepared. An acrylic co-polymer (Rheocoat 35 from Coatex) is added as a thickening agent to obtain a viscosity of about 1200 cP (measured according to Scan-P 50:84, but with a sample temperature of 34-40 °C). Further, the pH of the barrier coating composition is adjusted to about 8 using NaOH.

The barrier coating composition is applied with a roll which is dipped in a chest with the barrier coating composition and the excess is removed with a coating blade. The pressure and angle of the coating blade is adjusted such that the coat weight of the barrier coating is 8 g/m². The barrier coating surface is dried with IR-dryers, which allowing a fast setting of the coating colour. The drying continues with cylinders and hot air until the desired moisture level is obtained. Normally the finished product has a dry content of 92-95%.

The coated paper is the calendared in order to compress the coating and the fibers to make the surface and the fiber network even more closed and therefore more resistant to penetration of water. For the same reason rain will easier leave the surface of the sack.

### Sack preparation

Sacks (Sack 1 and Sack 2) are then prepared using the coated sack paper prepared according to the above as the outer paper ply and a commercial sack paper as the inner paper ply.

### Sack 1

Outer paper ply: Coated sack paper prepared according to the above
Inner paper ply: QuickFill^{®} Brown Plus (unbleached), marketed by BillerudKorsnäs AB (Sweden), see table 2
Free film: none
Deaeration concept: top deaeration according to figure 2

### Sack 2

Outer paper ply: Coated sack paper prepared according to the above
Inner paper ply: QuickFill^{®} Brown SE (unbleached), marketed by BillerudKorsnäs AB (Sweden), see table 2
Free film: none
Deaeration concept: top deaeration according to figure 2

**Table 2. Both papers of table 2 are formed from unbleached sulphate/kraft pulp from softwood**

| | QuickFill Plus Unbleached | QuickFill SE Unbleached |
|---|---|---|
| Grammage (g/m²) | 70 | 70 |
| Gurley (s) | 3 | 5 |
| Tensile strength MD/CD (kN/m) | 5.6/4.9 | 5.6/4.9 |
| TEA MD/CD (J/m²) | 215/240 | 215/240 |
| TEA index MD/CD (J/g) | 3.1/3.4 | 3.1/3.4 |
| Stretch MD/CD (%) | 6.0/8.0 | 6.0/8.0 |

### Deaeration test

The normalised MegaGurley flow according to Haver&Boecker (L/02) vs. pressure drop is tested for three different 25 kg sacks; Sack 1, Sack 2 and a commercially available reference sack. Sack 1 and Sack 2 are expected to show deaeration curves that are better than or comparable to the reference sack.

### Drop test for dry sacks

10 sacks according to Sack 1 or Sack 2 are filled with 24.9 kg cement each and tested in a drop test according to ISO 7965-1 (a constant drop height method, drop height = 1.2 m). The sacks are conditioned according to ISO 6599-1. The dimensions of each sack are 400 mm × 450 mm × 110 mm.

For each sack, the number of drops until failure is measured.

The result of the drop test is expected to be comparable to or better than the result obtained with a comparable "normal" sack with a slitted or perforated free film.

### Rain test

Sacks according to Sack 1 or Sack 2 are filled with about 25 kg of cement.

The filled sacks are exposed to rain conditions according to ISO 2875 for 2, 4, 6 or 8 hours. During the exposures, the sacks are oriented with the deaeration opening facing down.

After the exposures, the sacks are cut open and the cement is visually inspected. The condition of the cement is expected to be acceptable, also after 8 hours of exposure.

### Drop test after rain test

Sacks from the rain rest exposed to 2 hours of rain conditions are expected to survive several drops from a height of 80 cm without breaking. Sacks from the rain rest exposed to 8 hours of rain conditions are expected to survive several drops from a height of 40 cm without breaking.

## Claims

1. A coated paper for use in a sack, wherein:
the coated paper comprises a paper layer that is internal-sized with at least one hydrophobic size;
the sized paper layer is creped;
the sized paper layer is provided on a first side with a pre-coating layer and a barrier coating layer;
the pre-coating layer comprises binder and inorganic filler in a dry weight ratio of between 10:100 and 50:100;
the barrier coating layer comprises clay and synthetic rubber in a dry weight ratio between 1:1 and 2.4:1;
the sized paper is provided on a second side with a backside coating layer, which backside coating may have a coat weight of 1-5 g/m², such as 2-4 g/m²; and
the grammage according to ISO 536 of said coated paper is 75-140 g/m², such as 80-115 g/m²,
wherein the particle size (% < 2 µm) of the inorganic filler is 80 or less.

2. The coated paper according to claim 1, wherein the backside coating layer comprises starch and/or rubber, such as synthetic rubber, such as styrene-butadiene rubber.

3. The coated paper according to claim 1 or 2, wherein pre-coating layer comprises binder and inorganic filler in a dry weight ratio of between 15:100 and 40:100, such as between 20:100 and 35:100.

4. The coated paper according to any one of claims 1-3, wherein the inorganic filler comprises or consist of CaCO₃ pigment.

5. The coated paper according to any one of claims 1-4, wherein the particle size (% < 2 µm) of the inorganic filler is between 50 and 80, such as between 50 and 75, such as between 55 and 75.

6. The coated paper according to any one of claims 1-5, wherein the at least one hydrophobic size comprises AKD.

7. The coated paper according to any one of claims 1-6, wherein the coat weight of the pre-coating layer is 5-12 g/ m² and/or the coat weight of the barrier coating layer is 5-15 g/m².

8. The coated paper according to any one of claims 1-7, wherein the sized paper layer is a bleached paper layer.

9. The coated paper according to any one of claims 1-8, wherein the sized paper layer is creped by a Clupak or Expanda unit.

10. A sack for a hydraulic binder comprising an outer ply composed of the coated paper according to any one of claims 1-9.

## Patentansprüche

1. Beschichtetes Papier zur Verwendung in einem Sack, wobei:
das beschichtete Papier eine Papierschicht aufweist, die innen mit mindestens einer hydrophoben Leimung versehen ist;
die geleimte Papierschicht gekreppt ist;
die geleimte Papierschicht auf einer ersten Seite mit einer Vorbeschichtungsschicht und einer Sperrbeschichtungsschicht versehen ist;
die Vorbeschichtungsschicht Bindemittel und anorganischen Füllstoff in einem Trockengewichtsverhältnis zwischen 10:100 und 50:100 aufweist;
die Sperrbeschichtungsschicht Ton und synthetischen Kautschuk in einem Trockengewichtsverhältnis zwischen 1:1 und 2,4:1 aufweist;
das geleimte Papier auf einer zweiten Seite mit einer Rückseitenbeschichtungsschicht versehen ist, wobei die Rückseitenbeschichtung ein Beschichtungsgewicht von 1-5 g/m², beispielsweise 2-4 g/m², aufweisen kann;
und
die Grammatur gemäß ISO 536 des beschichteten Papiers 75-140 g/m², beispielsweise 80-115 g/m², beträgt,
wobei die Partikelgröße (% < 2 µm) des anorganischen Füllstoffs 80 oder weniger beträgt.

2. Beschichtetes Papier nach Anspruch 1, wobei die Rückseitenbeschichtungsschicht Stärke und/oder Kautschuk, beispielsweise synthetischen Kautschuk, beispielsweise Styrol-Butadien-Kautschuk, aufweist.

3. Beschichtetes Papier nach Anspruch 1 oder 2, wobei die Vorbeschichtungsschicht Bindemittel und anorganischen Füllstoff in einem Trockengewichtsverhältnis zwischen 15:100 und 40:100, beispielsweise zwischen 20:100 und 35:100, aufweist.

4. Beschichtetes Papier nach einem der Ansprüche 1-3, wobei der anorganische Füllstoff CaCO₃-Pigment aufweist oder daraus besteht.

5. Beschichtetes Papier nach einem der Ansprüche 1-4, wobei die Partikelgröße (% < 2 um) des anorganischen Füllstoffs zwischen 50 und 80, beispielsweise zwischen 50 und 75, beispielsweise zwischen 55 und 75, liegt.

6. Beschichtetes Papier nach einem der Ansprüche 1-5, wobei die mindestens eine hydrophobe Leimung AKD aufweist.

7. Beschichtetes Papier nach einem der Ansprüche 1-6, wobei das Beschichtungsgewicht der Vorbeschichtungsschicht 5-12 g/m² beträgt und/oder das Beschichtungsgewicht der Barrierebeschichtungsschicht 5-15 g/m² beträgt.

8. Beschichtetes Papier nach einem der Ansprüche 1-7, wobei die geleimte Papierschicht eine gebleichte Papierschicht ist.

9. Beschichtetes Papier nach einem der Ansprüche 1-8, wobei die geleimte Papierschicht durch eine Clupak- oder Expanda-Einheit gekreppt ist.

10. Sack für ein hydraulisches Bindemittel, aufweisend eine Außenlage aus dem beschichteten Papier nach einem der Ansprüche 1-9.

## Revendications

1. Papier revêtu destiné à être utilisé dans un sac, dans lequel :
le papier revêtu comprend une couche de papier qui est encollée à l'intérieur avec au moins une taille hydrophobe ;
la couche de papier encollé est crêpée ;
la couche de papier encollé est pourvue, sur une première face, d'une couche de pré-couchage et d'une couche de revêtement barrière ;
la couche de pré-couchage comprend un liant et une charge inorganique dans un rapport en poids sec compris entre 10:100 et 50:100 ;
la couche de revêtement barrière comprend de l'argile et du caoutchouc synthétique dans un rapport en poids sec compris entre 1:1 et 2,4:1 ;
le papier encollé est pourvu, sur une deuxième face, d'une couche de revêtement au verso, qui peut avoir un grammage compris entre 1 et 5 g/m², tel que compris entre 2 et 4 g/m² ;
et
le grammage selon la norme ISO 536 dudit papier revêtu est compris entre 75 et 140 g/m², tel que compris entre 80 et 115 g/m²,
dans lequel la taille des particules (% < 2 µm) de la charge inorganique est inférieure ou égale à 80.

2. Papier revêtu selon la revendication 1, dans lequel la couche de couchage dorsale comprend de l'amidon et/ou du caoutchouc, tel que du caoutchouc synthétique, tel que du caoutchouc de styrène et de butadiène.

3. Papier revêtu selon la revendication 1 ou la revendication 2, dans lequel la couche de pré-couchage comprend un liant et une charge inorganique dans un rapport en poids sec compris entre 15:100 et 40:100, tel que compris entre 20:100 et 35:100.

4. Papier revêtu selon l'une quelconque des revendications 1 à 3, dans lequel la charge inorganique comprend ou est constituée d'un pigment de CaCO₃.

5. Papier revêtu selon l'une quelconque des revendications 1 à 4, dans lequel la taille des particules (% < 2 µm) de la charge inorganique est comprise entre 50 et 80, telle que comprise entre 50 et 75, telle que comprise entre 55 et 75.

6. Papier revêtu selon l'une quelconque des revendications 1 à 5, dans lequel l'au moins une taille hydrophobe comprend de l'AKD.

7. Papier revêtu selon l'une quelconque des revendications 1 à 6, dans lequel le poids de la couche de pré-couchage est compris entre 5 et 12 g/m² et/ou le poids de la couche de couchage barrière est compris entre 5 et 15 g/m².

8. Papier revêtu selon l'une quelconque des revendications 1 à 7, dans lequel la couche de papier encollé est une couche de papier blanchi.

9. Papier revêtu selon l'une quelconque des revendications 1 à 8, dans lequel la couche de papier encollé est crêpée par une unité Clupak ou Expanda.

10. Sac pour liant hydraulique comprenant une couche extérieure composée du papier revêtu selon l'une quelconque des revendications 1 à 9.
